

July 27, 1965

G. A. MARSH ET AL

3,197,388

METHOD AND APPARATUS FOR ESTIMATING CORROSION RATE

Filed Dec. 22, 1961



INVENTORS  
GLENN A. MARSH  
BY ROBERT L. LITTLER  
*Edward W. Lang*  
ATTORNEY

3,197,388

METHOD AND APPARATUS FOR ESTIMATING  
CORROSION RATEGlenn A. Marsh and Robert L. Littler, Crystal Lake, Ill.,  
assignors to The Pure Oil Company, Chicago, Ill., a  
corporation of Ohio

Filed Dec. 22, 1961, Ser. No. 161,449

6 Claims. (Cl. 204—1)

This invention relates to a method and apparatus for determining the rate of corrosion of corrodible elements which form a multi-metallic, electrolytic corrosion system.

It has long been recognized that the rate of corrosion of one of a pair of dissimilar, corrodible metallic structures contacted by an electrolyte can be determined by measuring the zero-resistance current flow between the two structures. By application of Faraday's Law, the measured current can be converted to a rate of metal loss, expressed in inches of penetration per year, or other conventional units. Many more complex corrosion systems include a relatively large number of structures, all fabricated of different metals, some or all of which are electrically connected, and all of which are contacted by an electrolyte. The study of corrosion rates in such complex systems has, in the past, been approached by exposing individual couples to the electrolyte, so that the behavior of selected structures of the system with respect to each other may be evaluated. This method has proved to be less than satisfactory, because it fails to take into consideration the interaction of the numerous couples which comprise a complex electrolytic corrosion system, and the effect which such couples have upon each other.

The deficiencies of the methods of the prior art have been found to be especially apparent when it is desired to determine the efficiency of inhibitors used in complex electrolytic corrosion systems. For example, a gasoline engine and cooling system commonly will include members fabricated from cast iron, steel, copper, brass, solder, and aluminum, all of which are in contact with a cooling fluid which is an electrolyte. All of the aforesigned metals are connected in substantially short-circuit electrical relationship. Evaluating the rate of corrosion of one metal structure in the system, say an aluminum cylinder head, cannot very well be accomplished by determining the corrosion rates of aluminum elements disposed in a plurality of individual couples, including as second elements of the couples elements fabricated of various other metals of the system, due to the fact that interaction of the cells is not thereby taken into consideration. The evaluation of corrosion inhibitors by determining their effect upon various couples composed of selected metals of the system is highly unreliable, because it fails to take into consideration the effect which the passivation of one couple may have upon another couple. For example, the corrosion of an aluminum cylinder head may serve to passivate the cathodic tendencies of a copper radiator tube with respect to an iron engine member. Hence the use of a corrosion inhibitor which is selective for the passivation of aluminum, but not for iron, may actually result in a dramatic increase in the rate of corrosion of the iron member, and rapid failure thereof.

It is therefrom an object of this invention to provide a method and apparatus for determining the rates of corrosion of members of multi metallic-electrolytic corrosion systems. Another object of this invention is to provide a method and apparatus for determining the rate of corrosion of members of complex electrolytic corrosion systems, whereby the interaction of the various couples which comprise the system is taken into consideration.

The invention is best described with reference to the drawings, of which,

FIGURE 1 is a sectional view of a corrosion-measuring probe fabricated in accordance with this invention,

FIGURE 2 is a sectional view of an alternate corrosion probe, and

FIGURE 3 is a schematic diagram of an electric circuit which can be employed in conjunction with probes of FIGURES 1 and 2.

Referring to FIGURE 1, rod 10, which is fabricated of an electrically insulating, corrosion-impervious material, such as polyethylene, is threaded to receive support at 12 and is encompassed by specimens 14, 16, 18, and 20, which are spaced axially along rod 10. Electrical conductors 22, 24, 26, and 28 extend through rod 10 in electrically insulated relationship, and make connection to conductors 14, 16, 18, and 20, respectively. The junction between each conductor and specimen is preferably at the inside of the opening provided in the specimen, so that the connection is protected from exposure to the environment surrounding the assembly. Each specimen is fabricated of a different metal, and is made to provide an appropriate surface area. For example, where it is desired to fabricate an apparatus for simulating the conditions which exist in a gasoline engine and cooling system assembly, comprising a copper tube radiator of soldered construction, an iron engine block, and an aluminum cylinder head, the specimen 14 may be made of copper, the specimen 16 of solder, the specimen 18 of iron, and the specimen 20 of aluminum. The surface areas of the specimens are proportioned to the surface areas of the corresponding engine elements which are in contact with the electrolyte, i.e., the cooling fluid. For example, if the surfaces of the engine block in contact with the cooling fluid have five times the area of the surface of cylinder head in contact with the cooling fluid, the surface area of specimen 18 can be made 5 times as great as the surface area of specimen 20. For this purpose, the specimen 18 may be constructed with a plurality of fins, as shown.

In operation, the assembly of FIGURE 1 is immersed in exposure to an electrolyte, for example in exposure to a sample of cooling fluid taken from the cooling system of an internal combustion engine. By connecting the conductors 22, 24, and 26 together, and measuring the short-circuit current flow between conductor 28 and the connected conductors, as by placing a low-resistance ammeter therebetween, the rate of corrosion of the aluminum specimen can be measured, and thereby the rate of corrosion of the aluminum cylinder head estimated. Similarly, the rate of corrosion of the engine block can be estimated by connecting together conductors 22, 24, and 28, and placing an ammeter between conductor 26 and the connected conductors. In this manner, the rate of corrosion of each specimen, when under the influence of the corrosive environment and the effects of the remaining specimens, can be ascertained.

Referring to FIGURE 2, an alternate structure is shown. Block 30 is fabricated of an electrically insulating and corrosion-impervious material, such as a polyester resin. Tubular specimens 32, 34, and 36 are supported by base 30. Conductors 38, 40, and 42 pass through the block 30 and connect ends of the tubular specimens 32, 34, and 36, respectively.

Referring to FIGURE 3, a convenient switching and measuring arrangement for use in conjunction with above-disclosed assemblies is shown. Connection is made from the conductors of the test assemblies to the terminals, such as terminals 50, of switch assembly 52. The switch assembly includes a base 54, and a slide bar 56, both of which are made of an electrically insulating material. Conductive contact bars 58, 60, and 62 are attached to the slide bar 56. Contact 58 is connected to measuring circuit terminal 64, while contacts 60 and 62 are joined

together and connected to measuring-circuit terminal 66. Between the terminals 64 and 66, a variable resistance, a battery, and an ammeter are series-connected. A voltmeter is also connected across terminals 64 and 66. This circuit provides a very convenient means for measuring the zero-resistance current output of the specimens of the probe. The function of the variable resistance and the battery is to overcome the resistance of the ammeter measuring circuit. This is accomplished by setting the variable resistance so that the reading on the sensitive voltmeter is zero. In this situation, there is zero voltage drop across the ammeter measuring circuit. By moving slide 56 to the right or to the left, the short-circuit current between any selected specimen and the remaining specimens can be conveniently measured.

As a specific example of the method of this invention, and the use of the apparatus of this invention, it is desired to estimate the rate of corrosion of the aluminum member of a multi-metallic structure fabricated of four different metals, including aluminum, all of which are exposed to a corrosive environment. The corrosive environment comprises an aqueous salt solution. Four metal specimens are fabricated of metals identical to those which comprise the multi-metallic structure. The ratio of the area of the portion of the structure fabricated of a particular metal, and exposed to the corrosive environment, to the area of the specimen fabricated of the same metal is made constant for each portion of structure and corresponding specimen. This is done by adjusting the specimens to provide the required surface areas. The specimens are then suspended in a sample of the electrolyte, and electric lead wires, which themselves are insulated from the environment, are connected to each specimen. The lead wires coming from the various specimens, excluding that of aluminum, are connected together, and a zero-resistance ammeter is employed to measure the short-circuit current flow between the aluminum specimen and the other connected specimens. A current reading of 55 milliamperes is obtained. All of the lead wires except that connected to the steel specimen are then connected together, and the current flow between the steel specimen and the remaining specimens is measured and found to amount to 5 milliamperes. In each case, the direction of current flow is such as to indicate a corrosion of the aluminum and steel specimens. A corrosion inhibitor is then added to the electrolyte in which the specimens are immersed. The measurements are repeated with respect to the aluminum specimen and the steel specimen, and readings of 6 milliamperes and 8 milliamperes, respectively, are noted. From the foregoing tests, it is concluded that the inhibitor employed is effective to mitigate the corrosion of aluminum in the system under study, but that the inhibitor can be used only if a rate of corrosion of the steel corresponding to the eight millampere current can be tolerated.

The embodiments of the invention in which an exclusive property or privilege is claimed are defined as follows:

1. The method of estimating the rate of corrosion of a selected corrodible structural member in a multi-metallic, electrolyte-containing corrosion system including the selected member and a plurality of other electrically connected members fabricated of diverse metals comprising,

(a) exposing a specimen fabricated of the same metal

as said selected member to a body of electrolyte substantially identical with that of said corrosion system, (b) exposing a plurality of other specimens each of which is fabricated of the same metal, respectively, as one of the other members of said plurality to said body of electrolyte, each of all said specimens having a ratio of its surface area to the surface areas of the other specimens in contact with said body of electrolyte the same as the corresponding ratio of each member to the other members in contact with electrolyte in said corrosion system so as to provide a proportional duplicate of said corrosion system. (c) electrically connecting the specimens of said plurality in short circuit, and

(d) measuring the zero resistance current flow between said first specimen and the specimens of said plurality connected in short circuit.

2. A corrosion-measuring apparatus comprising,

(a) at least three corrodible specimens fabricated of different metals,

(b) means for supporting said specimens in electrically insulated relationship for exposure to a corrosive electrolyte,

(c) three electrical conductors connected to said three specimens, respectively,

(d) electrical switching means comprising at least three terminals to each of which is fastened one of said conductors,

(e) an electric circuit comprising in series an ammeter, a direct current source and a variable resistance and a voltmeter connected in parallel therewith,

(f) at least three separate electrical contact elements movable into and out of contact with said terminals,

(g) means connecting at least two of said contact elements in short circuit to one terminal of said circuit, and

(h) means simultaneously connecting a third contact means to the other terminal of said circuit.

3. An apparatus in accordance with claim 2 in which said means for supporting the specimens is fabricated of a corrosion-impervious, electrically insulating material.

4. An apparatus in accordance with claim 3 in which said support means comprises a rod adapted for insertion in a corrosive environment, and said specimens are spaced axially along the rod.

5. An apparatus in accordance with claim 4 in which said conductors extend within the rod from one end thereof to contact said specimens.

6. An apparatus in accordance with claim 5 in which each specimen is generally disc-shaped and provided with an opening through which the rod extends to internally contact and support the specimen.

#### References Cited by the Examiner

#### UNITED STATES PATENTS

|           |      |               |       |         |
|-----------|------|---------------|-------|---------|
| 2,805,191 | 9/57 | Hersch        | ----- | 204—1.1 |
| 2,903,405 | 9/57 | Sabins        | ----- | 204—197 |
| 3,050,371 | 8/62 | Dowson et al. | ----- | 204—1.1 |
| 3,051,631 | 8/62 | Harpin et al. | ----- | 204—195 |

WINSTON A. DOUGLAS, Primary Examiner.

JOHN R. SPECK, Examiner.